

July 7, 1942.

P. E. MAYER

2,288,727

TREATMENT OF TITANIUM-BEARING MATERIALS

Filed Nov. 13, 1939

2 Sheets-Sheet 1



INVENTOR.

PERRY E. MAYER

Kewis Hudson & Kent  
ATTORNEYS

July 7, 1942.

P. E. MAYER  
TREATMENT OF TITANIUM-BEARING MATERIALS

2,288,727

Filed Nov. 13, 1939

2 Sheets-Sheet 2



FIG. 2

INVENTOR.  
**PERRY E. MAYER**  
BY  
*Kris Hudson & Kent*  
ATTORNEYS

## UNITED STATES PATENT OFFICE

2,288,727

## TREATMENT OF TITANIUM-BEARING MATERIALS

Perry E. Mayer, Collingswood, N. J., assignor to  
The Sherwin-Williams Company, Cleveland,  
Ohio, a corporation of Ohio

Application November 13, 1939, Serial No. 304,144

10 Claims. (Cl. 23—88)

This invention relates to the treatment of titanium-bearing ores for the purpose of obtaining the titanium values in the form of water soluble compounds, and more particularly to the treatment of such ores as ilmenite and rutile to convert the titanium content into soluble fluoride compounds which may be converted by well known means and methods, such as those disclosed in the Svendsen Patents 2,042,434 and 2,042,435, into titanium hydrate of such purity and characteristic properties that pure pigment titanium dioxide may be produced therefrom.

It is the object of this invention to provide an improved method of treating the titanium ores, to obtain the soluble fluoride compounds, that will permit the use of simpler and less costly equipment and be more economical to operate than the fluoride methods heretofore known and used and, in consequence, effect a substantial reduction in the cost of producing the pigmentary titanium dioxide.

Titanium ores, for example, ilmenite and rutile, contain silicon compounds as impurities. The rutile contains iron compounds as impurities, whereas the ilmenite is composed of titanium and iron oxide compounds (probably in chemical combination) in varying proportions. These ores usually contain other impurities in small amounts such as heavy metals other than iron. The iron and heavy metals must be substantially entirely removed from the resulting titanium compounds so that the resulting titanium oxide may have the required whiteness and brilliancy. The silicon which is present in the ore reacts in a manner similar to titanium in the fluoride process, and the resulting titania contains this silicon in the form of silica.

The titanium-bearing raw material is digested with the ammonium fluoride salt, which term includes the bifluoride and compounds which under the conditions of reaction form ammonium fluoride, and the titanium, silicon, iron, and other heavy metal compounds react to form fluoride salts. The titanium and silicon form fluoride salts which are water-soluble under neutral or non-alkaline conditions. Because of the decomposition of at least a part of the ammonium fluoride to the bifluoride due to the instability of the ammonium fluoride at the reacting temperatures the final reaction product is non-alkaline, and the fluoride salts of titanium and silicon may be removed therefrom by leaching with water. The iron forms a double salt with ammonium fluoride which is soluble only to a slight degree in water and even less soluble in water containing ammonium fluoride in solution. However, this small amount of iron is sufficient to cause titania made therefrom, without further purification, to be off-color.

In carrying out the step of digestion of the

10 titanium-bearing ore with an ammonium fluoride salt, in accordance with Svendsen's method, it has been found in commercial practice that the control of corrosion of the apparatus is difficult. 5 The problem of corrosion has proven to be most acute in that part of the cyclic process dealing with the recovery of NH<sub>4</sub>F crystals or of a concentrated NH<sub>4</sub>F solution (50 to 60%) by evaporation of dilute NH<sub>4</sub>F solution (10 to 20%) obtained from the process.

15 I have found that the corrosive action of these NH<sub>4</sub>F or NH<sub>4</sub>F,NH<sub>4</sub>F,HF liquors can be controlled by the addition of finely pulverized ilmenite ore and carrying out the required evaporation of water vapor and NH<sub>3</sub> fume under pressures greater than atmospheric. I have observed that concentration of dilute NH<sub>4</sub>F solutions, containing 3% or more by weight of ilmenite, by evaporation of water vapor (steam) and NH<sub>3</sub> fume at a pressure of from 2 to 10 atmospheres, reduces the rate of corrosion of cold rolled steel from  $\frac{1}{2}$  to  $\frac{1}{5}$  the values observed when the concentration of the dilute NH<sub>4</sub>F liquors is carried out by boiling at atmospheric pressure or under vacuum in the absence of finely pulverized ilmenite. The practice of this discovery in accordance with my invention enables the use of equipment made from the less expensive corrosion-resistant alloys and greatly increases the effective life of the equipment used in the process.

20 25 30 35 Examination of the metal surfaces exposed to the action of the NH<sub>4</sub>F solution-ilmenite slurries during the simultaneous evaporation of the solution and attack of the ilmenite by the active NH<sub>4</sub>F salt at elevated pressures reveals that a coating, probably an iron fluoride, is formed on the metal surface, which serves as a protection from further corrosive action. The formation of this protective coating on the exposed metal surfaces and the consequent lessening of corrosion appears to be considerably facilitated by the presence of ilmenite in the NH<sub>4</sub>F solution and by the conditions resulting from carrying out the concentration-digestion step at pressures above 40 45 atmospheric.

Another feature of my invention that is of great importance has to do with the recovery of chemicals used in the process. I have found, in carrying out the cyclic process of digestion, boiling of the reaction mass, clarification of the titania liquor, precipitation of titania hydrate, and recovery of the active chemicals as described in the above-mentioned Svendsen patents, that a good recovery of these chemicals, fluorine, and 50 55 ammonia, is extremely difficult to obtain. This is due to many factors, some of which are the escape of fume from the digester, loss of NH<sub>4</sub>F and NH<sub>3</sub> during the concentration of the dilute NH<sub>4</sub>F liquor, escape of NH<sub>3</sub> into the air with 60 non-condensable gases (air) introduced into the

system and losses due to the extreme corrosive action of the digester fumes and the evaporator liquors. My invention has eliminated many of these factors and minimized others, and thus enables the recovery, with a minimum of effort, of a high percentage of the active agents used in each cycle. For example, by carrying out the evaporation of dilute  $\text{NH}_4\text{F}$  solution in a pressure vessel in the presence of the finely pulverized ilmenite ore, I eliminate the possibility of any fume escaping except as directed during the concentration of the solution; I prevent the access of non-condensable gases (air) to the system, and thus simplify the condensation and complete recovery of  $\text{NH}_3$  fume; I decrease the losses due to corrosion, as previously described, by repressing the corrosive action of the  $\text{NH}_4\text{F}$  liquor during concentration, and further, by elimination of the highly corrosive digester fumes. In addition to these items I have found that by my improved method I obtain a fume from the pressure vessel, during operation, containing not more than traces of  $\text{NH}_4\text{F}$ , whereas the fume obtained from the evaporation of dilute  $\text{NH}_4\text{F}$  solution to concentrated liquor under vacuum or at atmospheric pressure as in the Svendsen method has been found in practice to contain from 0.5 to 3% of  $\text{NH}_4\text{F}$ . Such extremely dilute  $\text{NH}_4\text{F}$  solutions are expensive to handle and increase the cost of the recovery system.

In performing the step of digestion of the titanium containing ore with an  $\text{NH}_4\text{F}$  salt or concentrated  $\text{NH}_4\text{F}$  aqueous solution as described in the Svendsen patents an excess of the fluoride salt is required primarily to attain high conversion of the titanium content of the ore to the form of water soluble titanium fluoride compounds, and, in addition, to assure an acidic condition in the subsequent leaching operation by the formation of ammonium acid fluoride in the digestion mass from the excess ammonium fluoride. Even with this excess present in the actual practice I have found that complete digestion of finely pulverized ilmenite ore is difficult of attainment, requires a long period of reaction, and frequently temperatures considerably in excess of  $175^\circ\text{C}$ . Furthermore the consistency of the reaction mass changes from a heavy fluid to a pasty condition and finally approaches a dry state during the course of the digestion. These physical states demand high power requirements to provide the necessary stirring or agitation of the reaction mass and afford very poor conditions for the efficient transfer of heat, thus making necessary very careful regulation of the heat input to prevent local overheating, loss of active fluoride constituents by vaporization and possible "freezing" of the digester by fusion of the reaction mass. These latter conditions are aggravated by the large excess of  $\text{NH}_4\text{F}$  salts found to be necessary to bring about complete conversion of the raw material.

I have found that these difficulties can be eliminated by the method of attack constituting my invention, resulting in considerable savings in time, power and heat requirements, and simplifying the control of the digestion step. By combining the digestion step with the recovery step of evaporation of the dilute  $\text{NH}_4\text{F}$  liquors obtained in the process, in accordance with the invention, I am able to secure substantially complete conversion of the titanium values in the raw materials to water soluble titanium fluoride compounds during the concentration of the dilute fluoride salt solution. By combining these mul-

tiple steps into one digestion step carried on in a pressure vessel at pressures greater than atmospheric I have found that satisfactory conversions of titanium-bearing ores can be obtained at temperatures as low as  $130^\circ\text{C}$ . to  $140^\circ\text{C}$ . The reaction mass in the pressure vessel remains in a very liquid state throughout the conversion, thus allowing very high heat transfer and low power requirements for agitation. Heating can be accomplished very efficiently through a jacketed vessel by steam or similar means. A further saving of heat is obtained by completing the conversion in the liquid state, thus materially decreasing the amount of water to be evaporated per cycle. Under certain conditions of operation it is possible to secure a substantially complete conversion of the titanium content of finely pulverized ilmenite ores into water soluble titanium fluoride compounds, and obtain a separation from the relatively insoluble iron fluoride compounds formed, by simple filtration, settling, or similar means without the introduction of any additional leach liquor or repulp water into the digested reaction mass. Titanium fluoride liquors so obtained are handled advantageously in the well known manner of the art to produce titanite hydrate of a high degree of purity which can be calcined to give titanium oxide having excellent pigment properties.

30 The control of the attack of the active fluoride compounds upon the titanium-bearing ore can be maintained easily by regulation of the several factors that have been found to influence the reaction. One of the more important of these factors is the pressure and corresponding temperature at which the reaction mass in the pressure vessel is maintained. The pressure is controlled very simply by regulating the heat input to the jacketed reaction vessel, the fume discharge from the vessel, or both.

Another important factor is the ratio of the active fluoride compounds (ammonium fluoride) to the titanium-containing material (ilmenite, rutile). I have found that I can obtain satisfactory conversion of ilmenite by my method of attack with a much smaller excess of  $\text{NH}_4\text{F}$  to ilmenite than it is necessary to use in the methods of attack at atmospheric pressure. For example, I am able to use less than 16 molecular parts (4 parts by weight of  $\text{NH}_4\text{F}$  to one of ilmenite) and obtain practically complete conversion of the ilmenite to fluoride compounds. I have also obtained satisfactory conversion using a ratio of less than 12 molecular parts (3 parts by weight of  $\text{NH}_4\text{F}$  to one of ilmenite). Under certain conditions I am able to obtain satisfactory results using a ratio of 2.5 parts by weight of  $\text{NH}_4\text{F}$  to one of ilmenite. This latter ratio approaches very nearly the theoretical quantities of  $\text{NH}_4\text{F}$  needed to attack and completely convert ilmenite into fluoride compounds according to the following equation:



Considerable economies in the operation of this cyclic process, particularly heat savings, can be made by operation of the digestion step with the smaller  $\text{NH}_4\text{F}$  ilmenite ratios which are made possible by my discovery. It has been found that the concentration of the  $\text{NH}_4\text{F}$  solution initially contacting the titanium-bearing material (ilmenite)

in the pressure vessel has a considerable influence on the subsequent pressure attack upon the ilmenite. Although the invention is not limited to an attack with NH<sub>4</sub>F solution of any particular concentration I am able by the control of other steps in the process to make available for the succeeding cycle an NH<sub>4</sub>F solution of the optimum concentration for pressure attack in the digestion step.

I have found further, that the pressure attack method of digestion can be operated to advantage on the counter-flow principle. By this modification of the process a portion or all of the water insoluble residue occurring from the leaching of the soluble titanium fluoride compounds can be contacted in a pressure vessel with a fresh portion of the dilute NH<sub>4</sub>F liquors available from the process and any small amounts of titanium compounds remaining in the residue be attacked and put in solution. The liquor from this secondary reaction mass containing small amounts of soluble titanium fluoride compounds is separated from the remaining insolubles by filtration, settling, or similar means and contacted in the same or another pressure vessel with a new quantity of titanium-bearing material (ilmenite) in the primary digestion step, the liquor obtained from this step being rich in soluble titanium fluoride compounds and suitable for further treatment for the production of titanium oxide of pigment qualities in the manner well known to the art. A division of the pressure attack digestion on the principle described enables the production of a titanium fluoride liquor well suited for further treatment in the production of titanium oxide pigment in the manner of the art and enables further a very high percentage of recovery (96 to 99+%) of the titanium content from the titanium-bearing materials. It may also be noted that this method of attack as just described allows the conversion process to be carried out with the minimum ratio of NH<sub>4</sub>F to ilmenite and thus provides the maximum of heat economy.

The apparatus that is preferred for carrying out the pressure digestion attack consists of a pressure vessel or autoclave suitably constructed of steel or alloy. This autoclave is equipped with an agitator of a type to produce efficient stirring in the body of the slurry during the attack and suitable means for charging and discharging the materials and for drawing off of fume. This vessel may be heated directly with gas or oil flame but I prefer to supply heat with steam, circulating oil or by similar means through a jacket.

Although I prefer to use a vessel equipped with some positive stirring device, it is not intended that the invention should be limited to the use of such type of stirring as I have found that the agitation of the slurry caused by the vigorous ebullition of fume during the attack may be sufficient to prevent the settling and baking of any of the heavier parts of the slurry.

The reacting materials may be introduced into the reaction chamber in a variety of ways. The aqueous fluoride solution may be introduced into the pressure vessel simultaneously with the ore, or the ore may be suspended in solution of the fluoride and the suspension fed into the autoclave. My preferred method is to introduce a suspension of all of the ore with a portion of the aqueous fluoride solution into the autoclave and feed in the remainder of the fluoride solution re-

quired for the attack during the course of the digestion.

In the accompanying drawings:

Fig. 1 is a diagrammatic illustration of apparatus for practicing the invention in a two-stage digestion method.

Fig. 2 is a flow sheet illustrating the various steps in the recovery of the titanium dioxide from the ores.

The following is a specific example for carrying out the digestion in two steps, a primary and secondary, according to this invention, although it is to be understood that said invention is not limited to the exact conditions set forth in this description.

#### Secondary stage

Referring to Fig. 1 of the drawings, 700# of 20% NH<sub>4</sub>F solution is charged into the steam jacketed autoclave 10, equipped with a stirrer 11, pressure gauge 12, and thermometer well 13, by means of the pipe 14, pump 15 and supply pipe 16. A fume discharge pipe is indicated at 17 and provided with a control valve 18. A discharge pipe for the slurry is indicated at 19. A charge of 125# of iron fluoride filter cake obtained from the primary digestion, hereinafter described, and containing from 8 to 16% of undigested or partially digested ilmenite is then added to the autoclave 10, through the manhole 19'. The vessel is sealed and steam at 100# gauge pressure is admitted to the jacket by means of the pipe 20 and control valve 21. The condensation in the jacket is discharged through the pipe 22 which is controlled by the valve 23. When the pressure within the autoclave reaches 75# on the gauge 12 the fume discharge valve 18 is opened and regulated to permit a continuous discharge of vapors at 75# pressure. The stirrer 11 is operated while the digestion is in progress.

An additional 300# of 20% NH<sub>4</sub>F solution is fed into the autoclave during the course of the digestion by means of pump 15' which is preferably a chemical proportioning pump. The digestion is continued until approximately 500# of water containing from 4 to 6% NH<sub>3</sub> has been vaporized and discharged through pipe 17. The supply of steam to the heating jacket is then cut off by closing valve 21 and the pressure in the autoclave allowed to fall to normal atmospheric pressure. The total time required for this secondary digestion step is about three hours. The temperature of the reaction mass in the autoclave during this digestion will be approximately 150° C. After the autoclave pressure has dropped to atmospheric, the slurry remaining, 625#, is discharged by pipe 19 and pump 24 to a filter 25 and the filter cake, 125#, is washed free from occluded titanium fluoride salts with 166# of very dilute NH<sub>4</sub>F solution, which may be supplied through pipe 26, the wash liquor being allowed to pass along with the mother liquor to a storage tank 27, by closing valve 28 and opening valve 29, to make 666# of approximately 30% NH<sub>4</sub>F.NH<sub>4</sub>F.HF solution. The iron fluoride filter cake, free of ilmenite and soluble titanium fluoride compounds, is removed from filter 25 and passed along to another step in the cyclic process for the recovery of fluorine as at 20% NH<sub>4</sub>F solution by known methods.

#### Primary stage

The 30% acid liquor, 666#, is withdrawn from tank 27 and charged into the autoclave by means of pipe 30 and pump 15, the valve 31 being open and the valve 32 closed. 100# of finely pulver-

ized ilmenite is added through the manhole 19 and the primary digestion carried out in a similar manner at 75# gauge pressure. During the reaction an additional 500# of 20% NH<sub>4</sub>F solution is fed by pump 15 into the autoclave from the supply 16 at the same rate as fume is discharged. The heating of the autoclave is discontinued when about 891# of steam containing approximately 6% NH<sub>3</sub> has been driven off through pipe 17, and the pressure is then allowed to fall to atmospheric. 452# of water containing small percentages of NH<sub>4</sub>F and NH<sub>3</sub> obtained as filter washes from the general cyclic process is then added to the digested autoclave slurry and the thinned slurry is then, by means of the pump 24, passed through the filter 25. The filter cake, 125#, is then used as described above, for the secondary digestion. The liquor, 712#, containing about 8% of TiO<sub>2</sub> in the form of soluble fluorides is passed from the filter 25 through pipe 33 to the treating system (not shown) for conversion to titanium hydrate. The 20% NH<sub>4</sub>F solution used in the digestion is recovery liquor obtained from the treating system after the precipitation and filtration of titania hydrate from the treated titania liquor. A heating period of about five hours is required for the primary digestion.

In order to reduce corrosion in the apparatus it is advisable to use a second autoclave 34 which is similar in all respects to the autoclave 10 with piping preferably provided in parallel arrangement so that the pumps 15 and 24 may be used for either autoclave. It will be understood, however, that each autoclave may have its own independent pumps and piping system but the arrangement shown in Fig. 1 is of advantage in reducing the amount of equipment required. With the two autoclaves the primary digestion described above may be carried out in one while the secondary digestion is being carried out in the other, thereby greatly increasing the capacity of the plant, and after each digestion the autoclaves may be reversed so that they will be used alternately for the primary and secondary digestions.

The following is a second specific example to illustrate how the digestion may be carried out in one step according to this invention.

Example.—950# of 20% NH<sub>4</sub>F solution is charged to the autoclave, 100# of finely pulverized ilmenite added, the vessel sealed and heated by passing steam at 100# gauge pressure into the jacket. When the pressure inside the autoclave has reached 75# gauge pressure corresponding to about 150° C., the fume discharge valve is opened and regulated to permit the continuous discharge of steam and NH<sub>3</sub> vapor at 75# pressure. An additional 1000# of 20% NH<sub>4</sub>F solution is pumped into the autoclave during the digestion at about the same rate as the fume is discharged. The digestion is completed and the heating discontinued when about 1475# of fume (water and NH<sub>3</sub>) have been discharged. The digested slurry remaining in the autoclave is diluted with about 362# of filter wash liquors, recovered in the process, and passed to the filter. The iron fluoride filter cake obtained, 125#, is washed free of soluble titanium fluoride compounds and then transferred to another step in the process for the formation of hydrated iron oxide and the recovery of the fluorine as a 20% NH<sub>4</sub>F solution. The mother liquor from the filter, about 712#, containing approximately 8% of TiO<sub>2</sub> in the form of a soluble titanium fluoride compound is passed

to the treating system for further purification, according to the art, and conversion to titania hydrate suitable for calcination to titanium oxide having excellent pigment properties.

It is not intended that the foregoing specific examples of the attack of ilmenite ore according to the invention should limit the scope of said invention. I have applied the pressure attack method on several types of ilmenite ores and other titanium containing materials, and have investigated the digestion of ilmenite over a range of pressures varying from atmospheric to 9 atmospheres, 135# gauge, and have obtained improved results, in comparison with prior methods, in all cases. I have also practiced the invention in the digestion of ilmenite under conditions involving (a) changing of the relative amounts of NH<sub>4</sub>F solution and ilmenite used or as I designate this—the fluorine to ilmenite ratio, (b) changing of the amount of fume discharged during the digestion or as I designate this—the percent of fluorine in the final digested slurry, (c) changing of the initial concentration of the NH<sub>4</sub>F solutions contacting the ore during digestion, but the foregoing specific examples represent the preferred procedures. From the standpoint of operating efficiency and results the two stage digestion method as described in the first specific example is preferred.

By employing the counter flow principle as illustrated, I am able, most effectively, to utilize the inherent advantages of the invention resulting from attack at elevated pressures and the combination of digestion with the concentration of dilute NH<sub>4</sub>F liquors. I obtain by this method the most nearly complete digestion with the lowest fluorine to ilmenite ratio, the largest heat economies, and the most efficient use of weak filter wash liquors recovered in the process.

I have mentioned above that the extreme fluidity of the reaction mass in the autoclave, even in the final stages of digestion, enables me to obtain a very efficient transfer of heat at relatively low power cost for agitation. I should point out also, that the fine dispersion of the ilmenite particles throughout the reaction mass obtained by mild agitation provides an ideal condition for the attack of the particles by the active fluoride salt. This suspension of the pulverized ilmenite in the NH<sub>4</sub>F solution tends to become more permanent as the digestion progresses and shows less tendency to settle out, thus approaching to the most favorable condition for complete reaction.

In addition to this physical condition favorable for rapid and complete digestion, there is a chemical reaction promoted by the pressure attack method that aids the rapid digestion of the titanium-bearing ore. This reaction is the dissociation of NH<sub>4</sub>F to NH<sub>4</sub>HF according to the equation: 2NH<sub>4</sub>F = NH<sub>4</sub>F.HF + NH<sub>3</sub>.

This reaction proceeds quite slowly at temperatures below 100° C., but becomes quite rapid at higher temperatures in the neighborhood of 140–150° C. I believe that the actual attack on the ilmenite ore during its digestion is carried on largely by the more chemically active NH<sub>4</sub>HF salt rather than by the neutral NH<sub>4</sub>F salt. Hence, quickly raising the temperature of the reaction mass to about 140–150° C. and maintaining this temperature by carrying out the entire digestion under a corresponding pressure in a pressure vessel, accelerates the rate of digestion by increasing the rate of formation of the active agent (NH<sub>4</sub>HF salt). By maintain-

ing the finely pulverized ilmenite ore in a highly dispersed condition throughout the fluid reaction mass, ideal conditions are provided for the rapid digestion of said ore by the bifluoride salt as fast as the latter is formed. The NH<sub>3</sub> vapor formed by the decomposition of the NH<sub>4</sub>F salt is discharged continuously from the pressure vessel along with steam as the digestion progresses.

This explanation of the probable mechanism of the digestion reaction also accounts for the lower ratio of NH<sub>4</sub>F to ilmenite required for digestion. According to the chemical equations for the reactions, as previously given, and subscribed to by Svendsen in his Patent No. 2,042,435, ten molecular parts of NH<sub>4</sub>F are required to completely digest one molecular part of ilmenite, or approximately 2½ parts by weight of NH<sub>4</sub>F to one part by weight of ore. As stated above I am able to obtain by my pressure digestion method a substantially complete digestion of ilmenite with as low as 2½ parts by weight of NH<sub>4</sub>F, showing that all of the available NH<sub>4</sub>F is utilized in the digestion process. This is not possible in the Svendsen process since he recommends the use of from 3 to 4 parts by weight of NH<sub>4</sub>F to one of ilmenite in order to obtain a satisfactory digestion of the ore. This considerable excess of NH<sub>4</sub>F required for digestion in the Svendsen process is necessary because of the difficulty in obtaining a thorough dispersion of the reacting materials in the pasty to dry reaction mass and because of the high temperatures reached in the said reaction mass during the final stages of digestion, which, since the digestion is carried out at atmospheric pressure, causes the vaporization and loss of appreciable quantities of unreacted NH<sub>4</sub>F or NH<sub>4</sub>F.HF.

By carrying out the digestion under pressures greater than atmospheric, according to my invention, I prevent the vaporization of any of the active constituents, NH<sub>4</sub>F or NH<sub>4</sub>F.HF, from the reaction mass, and thus make them available for complete utilization. In addition, the complete dispersion of the reacting materials obtained in the fluid condition of the reaction mass aids in securing a complete reaction with the theoretically necessary quantities of materials.

In the specification and claims, except where otherwise specifically stated, I intend to use the term ammonium fluoride in a generic sense to include the bi-fluoride as well as the fluoride.

Having thus described my invention, I claim:

1. In the herein-described process of recovering titanium compounds from titaniferous ore, the step which consists of treating the finely ground ore with a reactive aqueous fluoride solution under a pressure above atmospheric and at the boiling temperature of the reaction mass at said pressure and maintaining the reaction mass in a highly liquid state throughout the period of the reaction.

2. In the herein-described process of recovering titanium compounds from titaniferous ore, the step which consists of mixing the finely ground ore with a sufficient quantity of aqueous ammonium fluoride solution to form a highly liquid reaction mass and boiling said reaction mass under a pressure above atmospheric and under conditions in which the water and ammonia that are driven off are replaced by additional liquid to maintain the reaction mass in a liquid state throughout the period of the reaction.

3. In the herein-described process of recovering

- titanium compounds from titaniferous ore, the step which consists of mixing the finely ground ore with a sufficient quantity of relatively dilute aqueous fluoride solution to form a highly liquid reaction mass and boiling said reaction mass under a pressure above atmospheric and under conditions in which there is effected simultaneously a reaction of the fluoride with the metallic content of the ore to form metal fluorides, and 5 a concentration of the fluoride solution by the continuous withdrawal of the vapors that are boiled off and continuous addition of sufficient additional aqueous fluoride solution to maintain a constant reaction volume.
- 10 4. In the herein-described process of recovering titanium compounds from a titaniferous ore, the step which consists of boiling a liquid reaction mass of aqueous fluoride solution and the finely divided ore under a pressure above atmospheric and maintaining the liquidity of the reaction mass throughout the period of the reaction by the addition of aqueous fluoride solution to replace water that is evaporated therefrom.
- 15 5. In the herein-described process of recovering titanium compounds from a titaniferous ore, the step of concentrating relatively weak ammonium fluoride solutions by boiling the same in the presence of ilmenite and under a pressure of from 2 to 10 atmospheres.
- 20 6. In the herein-described process of recovering titanium compounds from a titaniferous ore, the step which consists in the production of aqua ammonia from relatively weak ammonium fluoride solutions by reaction with ilmenite under a pressure of from 2 to 10 atmospheres and at the boiling temperature corresponding to such pressure.
- 25 7. The herein-described two-stage process of recovering titanium compounds from titaniferous ore, the first stage of which consists in treating a quantity of finely pulverized ore with ammonium fluoride solution of greater than 20% concentration under a pressure of from 2 to 10 atmospheres and at the boiling temperature corresponding to such pressure, adding ammonium fluoride solution in sufficient quantity to make up for the water vapor and ammonia that are driven off and maintain the reacting mass in the form of a slurry, filtering the slurry, treating the filtrate to recover titanium compounds contained therein, then as the second stage of the process treating the filter cake with additional ammonium fluoride solution of about 20% concentration under a pressure of from 2 to 10 atmospheres and at the boiling temperature corresponding to such pressure, adding ammonium fluoride solution in sufficient quantity to make up for the water vapor and ammonia that are driven off and maintain the reacting mass in the form 30 of a slurry, filtering the slurry, and utilizing the filtrate in the first stage of the treatment of another quantity of finely pulverized ore.
- 35 8. In the herein-described cyclic process of recovering titanium products from titaniferous ores, the steps of adding to the finely pulverized ore in a pressure vessel provided with an agitator an aqueous solution of titanium and ammonium fluorides obtained from a previous cycle and of greater than 20% concentration and containing insufficient quantity of ammonium fluoride to effect complete digestion of said ore, further adding, while maintaining the solution under a pressure corresponding to a boiling point above about 150° C., a quantity of weak

ammonium fluoride liquors of less than 20% concentration to simultaneously effect partial conversion of said ore to fluorides and concentration of the weak ammonium fluoride liquors, separating the partially digested ore from the solution of titanium-ammonium-fluoride and treating said partially digested ore under similar conditions with sufficient aqueous ammonium fluoride at about 20% concentration to effect conversion to fluorides, and separating the titanium-ammonium-fluoride solution containing more than about 20% ammonium fluoride from the solids for use in the next cycle under the conditions herein described with reference to the first mentioned aqueous solution.

9. In the herein-described cyclic process of recovering titanium products from titaniferous ores, the steps of adding to the finely pulverized ore in a pressure vessel provided with an agitator an aqueous solution of titanium and ammonium fluorides obtained from a previous cycle and of greater than 20% concentration and containing insufficient quantity of ammonium fluoride to effect complete digestion of said ore, further adding, while maintaining the solution under a pressure corresponding to a boiling point above about 150° C., a quantity of weak ammonium fluoride liquors of about 5% or less concentration to simultaneously effect partial conversion of said ore to fluorides and concentration of the weak ammonium fluoride liquors, separating the partially digested ore from the solution of titanium-ammonium-fluoride and treating under similar conditions with sufficient aqueous ammonium fluoride at about 20% concentration to effect conversion to fluorides, and separating

the titanium-ammonium-fluoride solution, containing more than about 20% ammonium fluoride from the solids for use in the next cycle under the conditions herein described with reference to the first mentioned aqueous solution.

10. In the herein-described cyclic process of recovering titanium products from titaniferous ores, the steps of adding to the finely pulverized ore in a pressure vessel provided with an agitator an aqueous solution of titanium and ammonium fluoride obtained from a previous cycle and of greater than 20% concentration and containing insufficient quantity of ammonium fluoride to effect complete digestion of said ore, further adding, while maintaining the solution under a pressure corresponding to a boiling point above about 150° C., and while simultaneously releasing sufficient fume to reduce the quantity of water and the free NH<sub>3</sub> liberated, a quantity of weak ammonium fluoride liquors of less than 20% concentration to simultaneously effect partial conversion of said ore to fluorides and concentration of the weak ammonium fluoride liquors, separating the partially digested ore from the solution of titanium-ammonium-fluoride and treating under similar conditions with sufficient aqueous ammonium fluoride at about 20% concentration to effect its conversion to fluorides, separating the titanium-ammonium-fluoride solution containing more than about 20% ammonium fluoride from the solids for use in the next cycle under the conditions herein described with reference to the first mentioned aqueous solution.

PERRY E. MAYER.